

## UNITED STATES PATENT OFFICE.

HENRY C. KIRK, OF ROLAND PARK, AND GEORGE H. DUMLER, OF BALTIMORE,  
MARYLAND.

## ALLOY.

No Drawing. Original application filed May 23, 1919, Serial No. 299,364. Divided and this application filed February 19, 1920. Serial No. 359,803.

To all whom it may concern:

Be it known that we, HENRY C. KIRK and GEORGE H. DUMLER, citizens of the United States of America, the former residing at 5 Roland Park, Baltimore County, Maryland, and the latter in the city of Baltimore, State of Maryland, have invented certain new and useful Improvements in Alloys, of which the following is a specification.

10 The present application is a division of our application No. 299,364, filed May 23, 1919, which is in part a continuation of our applications 255,040, filed September 21, 1918, and 260,159, filed October 29, 1918.

15 The invention relates to an alloy of copper, nickel and iron substantially in the proportion of 10% iron, 20% nickel and the balance, approximately 70%, copper. The alloys which we have produced in accordance 20 with the disclosure of the foregoing applications comprise a series, having a considerable range and the object of the present application is to cover the alloys of approximately the proportions above pointed out, 25 and variations of this alloy having similar proportions and substantially the same properties.

An alloy which we have made, and which we consider to be included within this definition, contains 18% nickel and 10% iron, the balance being copper. It is a white material resembling silver in appearance, very tenacious, of high tensile strength and with high ductility. It can be rolled, readily 35 spun and drawn into tubes, also it can be stamped into any desired shapes.

A metal having the composition of 22½% nickel, 11½% iron and the balance copper shows in the Brinell test for hardness #121 40 and #126. It has a specific gravity of 865 and a weight per cubic inch of 0.31 pounds. It can be rolled from a thickness of .500 to .009 inch without annealing. Hard rolled, it has a tensile strength of 106,000 to 113,400 45 pounds per square inch, elastic limit 94,500 to 107,000 pounds per square inch, elongation in two inches hard rolled two to four per cent, annealed it has a tensile strength of 73,340 to 86,100 pounds, elastic limit 47,000 50 to 51,000 per square inch, elongation 30 to 26%. As a sand casting, it has a tensile

strength of 40,000 pounds per square inch, and an elastic limit of 30,000 pounds per square inch.

This metal is of a white color resembling 55 silver in appearance. It is non-corrosive, most organic acids have no effect on it, and it is remarkably well adapted as a substitute for silver or for any purpose where strength, durability and appearance are important. 60

Comparing it to German silver, it is much whiter, stronger and not as easily oxidizable. An alloy containing 20% nickel, 8½% iron, the balance being copper, which is a good 65 alloy for sheet material, wire and so forth, as a sand casting, without annealing, shows an elastic limit of 37,730 pounds per square inch, tensile strength of 40,500 pounds per square inch, and an elongation of 4% in two inches. The same material cold-rolled 70 shows an elastic limit of 107,000 pounds per square inch, a tensile strength of 113,400 pounds per square inch, and an elongation of 3% in two inches. Annealed it shows an elastic limit of 89,000 pounds per square 75 inch, a tensile strength of 73,340 pounds per square inch and an elongation of 30% in two inches.

In each instance we have referred to the percentage of nickel and iron. It is understood 80 that the balance of 100 per cent is copper.

In the production of this alloy, according to the preferred development of the industry, the nickel has served as a carrier for introducing the iron into the copper. Investigations show that 2% of nickel will carry 10% to 15% iron into the alloy; that is, 2% of nickel is sufficient to make it possible to form an alloy of copper, nickel and iron, 2% 85 nickel, 10% iron and the balance copper. However, the carrying power of nickel, i. e., its availability for introducing iron into copper is not utilized to the full extent in the alloy herein disclosed. The proportions 90 of applicants' preferred alloy are recited on page 1, paragraphs 2, 3, 4 and on page 2, paragraph 2, beginning line 12.

The use of a scavenger or oxidizing element as ferrosilicon or manganese has 100 been found desirable in all instances. The simplest method of making the alloy out of

common commercial material is by dissolving iron in a molten mixture of nickel and copper, preferably at the melting point of the mixture, which is closely related to the 5 melting point of nickel, the nickel having a solvent effect on the iron, which alone has a higher melting point than nickel, and cannot be directly combined with copper.

What we claim and desire to secure by  
10 Letters Patent is:

1. An alloy containing copper, nickel and iron in approximately the proportion of

20% nickel, 10% iron and the balance copper.

2. An alloy of copper, nickel and iron, 15 substantially as described.

Signed by us at Baltimore, Maryland,  
this 18th day of February, 1920.

HENRY C. KIRK.  
GEORGE H. DUMLER.

Witnesses:

ZELLA KUHN,  
SELMA STERN.